

Patented June 17, 1924.

1,497,889

# UNITED STATES PATENT OFFICE.

WILLIAM BERTIN BROOKFIELD, OF SYRACUSE, NEW YORK.

## METHOD OF MAKING HIGH-SPEED STEEL.

No Drawing.

Application filed June 16, 1922. Serial No. 568,864.

To all whom it may concern:

Be it known that I, WILLIAM B. BROOKFIELD, a citizen of the United States of America, and a resident of Syracuse, in the county of Onondaga, in the State of New York, have invented new and useful Improvements in Methods of Making High-Speed Steel, of which the following is a full, clear, and exact description.

10 This invention relates to the manufacture of steel for high-speed metal-cutting tools and analogous uses requiring a high degree of inherent and uniform resistance to wear and breakage.

15 The methods most commonly employed for producing steel of this character are: the "electric" and the "crucible" and it is well known by those skilled in this art that "steels" produced by the "electric" processes

20 under the most skillful treatment contain varying quantities of non-metallic substances or inclusions which may or may not be disclosed under the usual microscopic or chemical tests but nevertheless destroy the

25 perfect homogeneity of the product and frequently appears in the completed tools in the form of "chipping" or breakage when subjected to more or less stress and strain in use.

30 In the "crucible" process, the materials are melted in a considerable number (24 or more) crucibles in the same furnace and it is found to be practically impossible to obtain the same quality of steel in the several

35 units due to the inability of applying a uniform melting heat to the separate units or to different parts of the same unit.

Furthermore, while the "electric" melting process has the advantage of producing a more uniform grade of steel than that produced by the "crucible" process, the materials must be treated in relatively large masses and cast into correspondingly large ingots which must be "cogged" or reduced into smaller sections before they can be worked into stock.

40 This "cogging" involves not only considerable time and labor but also requires frequent heating and reheating of the ingot and its sections in working it into the required stock and results in considerable loss by oxidation and causes more or less decarbonization of the stock, all of which is expensive to the manufacturer and detrimental to the purchaser.

45 On the other hand, the "crucible" process

has an advantage over the "electric" process in that the molten metal may be cast into relatively small molds which may be readily worked into the required stock without decarbonization or excess loss by oxidation.

50 The main object of my process is to obtain the advantages of both the "electric" and "crucible" processes and at the same time to eliminate their disadvantages and thereby to produce a better and more uniform grade of steel than can be produced by either of those processes.

55 This is accomplished by first reducing a relatively large quantity of the raw materials to a molten state in an electric furnace under proper slag conditions and sufficient temperature to assure a product of maximum homogeneity and then transferring this highly homogeneous molten metal

60 to a series of heated crucibles in a suitable crucible furnace and subjecting these units to a temperature of approximately 2850 degrees F. for a period of about twenty to thirty minutes to allow the non-metallic inclusions to collect at the surfaces where they are skimmed off and finally casting the molten metal directly from the crucibles into relatively small molds ready to be worked into the desired stock.

65 By this process, I am enabled to take advantage of the less expensive melting of large quantities of the cheaper grades of base materials in the electric furnace and thereby to secure a molten steel product

70 having a more uniform chemical analysis than is possible by the "crucible" process, while the additional heat treatment of this molten product in reduced quantities in the

75 separate and relatively small crucible units greatly assists in securing a uniform temperature in all of the units and permits the elimination of the non-metallic inclusions

80 which are unavoidably present in the electric furnace product so that the product resulting from the two heat treatments is not only free from non-metallic substances but

85 possesses a maximum degree of homogeneity and uniformity of chemical analysis required for various tools and other uses and reduces

90 to a minimum the liability of "chipping" or

95 breaking of the tools when put to use.

100 The real merit of the invention as distinguished from the prior art is that after the electric furnace product has been introduced

105

110 into the crucibles, a sufficient amount of slag is introduced into the molten metal in the

crucibles to seal the same against oxidizing influences of the air or furnace heat during which time and for a definite period of say twenty (20) or thirty (30) minutes, this molten metal in the crucible units is maintained at approximately its original temperature (electric furnace temperature) to allow the non-metallic inclusions, which were in the original electric furnace product to rise to the surface and to unite with the added slag and eventually be skimmed off before pouring, thereby leaving a better and cleaner product substantially free from non-metallic inclusions and therefore of more uniform grade or quality than has heretofore been practicable under either of the methods herebefore mentioned.

What I claim is:

The herein described method of making steel consisting in reducing a relatively large mass of the base materials to a molten state in an electric furnace, transferring this molten metal into a series of relatively

smaller heated crucibles in a crucible furnace, adding a sufficient amount of extra slag to the molten metal in the crucibles to seal the same against oxidizing influences of the air or furnace heat and to expedite the collections of the non-metallic inclusions on the surface of the molten metal, retaining the molten metal in the crucible at approximately its original temperature and for a period of time as will cause the non-metallic inclusions therein to rise to the surface and to unite with the added slag, then skimming off the slag with the non-metallic inclusions therein and finally pouring the molten metal from the crucibles into relatively small molds.

In witness whereof I have hereunto set my hand this 12th day of June, 1922.

WILLIAM BERTIN BROOKFIELD.

Witnesses:

H. E. CHASE,  
M. C. RILL.